

# UNITED STATES PATENT OFFICE.

FRANZ MUELLER, OF ZURICH, SWITZERLAND.

## PROCESS OF WEIGHTING SILK WITH HÆMATOXYLIN.

1,207,784.

Specification of Letters Patent.

Patented Dec. 12, 1916.

No Drawing.

Application filed November 29, 1913. Serial No. 803,861.

To all whom it may concern:

Be it known that I, FRANZ MUELLER, a citizen of Germany, residing at 18 Ottikerstrasse, Zurich 6, Switzerland, have invented 5 a new and useful Process of Weighting Silk with Hæmatoxylin; and I do hereby declare the following to be a full, clear, and exact description of the same.

This invention relates to the process of 10 weighting silk with hæmatoxylin.

It is known that hæmatoxylin has been employed as a means for loading or weighting silk. For this purpose the method has always been to subject the silk to preliminary treatment of one kind or another and 15 then to manipulate it in a hot bath of hæmatoxylin and soap.

It has now been found that an addition of 20 water soluble phosphates to the hæmatoxylin bath presents sundry advantages, whether in presence of soap or without soap. In this way a considerably higher increase 25 of weight can be effected without other disadvantages, and the weighted silk is made firmer and gets a better grip by the proposed means.

Example: The boiled or scoured silk is preferably weighted beforehand by the generally known methods with zinc hydrate, 30 phosphate or phosphate-silicate; it is then manipulated at about 50° C. in a warm bath of, for example, 100 parts hæmatoxylin and 50 parts or more of sodium phosphate with a gradual raising of the temperature of the 35 bath, until the desired weighting is reached. The bath can be preserved and after addition of fresh hæmatoxylin and phosphate can be used again, which is not practicable if soap is employed. The quantities of 40 hæmatoxylin and phosphate depend upon the previous treatment of the silk and upon the weighting desired. Soap may also be added to the above mentioned bath. The nearer this preliminary weighting—viz. the 45 treatment with zinc-phosphate preceding that with hæmatoxylin—is equal to the required final weighting, the less hæmatoxylin and sodium phosphate will be added and the less will be the percentage of sodium phosphate 50 relatively to hæmatoxylin, while on the other hand, the greater the difference is

between the preliminary and final treatments, the more hæmatoxylin and phosphate is added. In this case again there is obtained by the addition of phosphate and 55 with the same quantity of hæmatoxylin a higher weighting than when only hæmatoxylin and soap are used. Consequently the proposed means, viz. the presence of soluble phosphate salt in the weighting bath 60 itself, means a valuable improvement even in the known processes of weighting by means of hæmatoxylin and soap.

I claim:

1. A process consisting in treating silk 65 with a bath of hæmatoxylin and sodium phosphate.

2. A process consisting in treating silk with a bath of hæmatoxylin and sodium phosphate at about 50° C. 70

3. A process consisting in treating silk with a bath of hæmatoxylin and sodium phosphate at about 50° C.; and increasing the temperature of the bath.

4. A process of weighting silk consisting 75 in treating the silk with a bath of 100 parts hæmatoxylin and 50 parts sodium phosphate at about 50° C.; and increasing the temperature of the bath.

5. A process of weighting silk consisting 80 in manipulating the silk at about 50° C. in a warm bath of 100 parts hæmatoxylin and 50 parts sodium phosphate; and gradually increasing the temperature of the bath.

6. A process of weighting silk consisting 85 in giving the silk a preliminary weighting; manipulating the silk at about 50° C. in a warm bath of 100 parts hæmatoxylin and 50 parts sodium phosphate; and gradually increasing the temperature of the bath until 90 the desired weighting is reached.

7. A process of weighting silk by means 95 of hæmatoxylin in which process soluble phosphates are present in the hæmatoxylin itself and soap is added.

In testimony whereof, I have signed my name to this specification in the presence of two subscribing witnesses.

FRANZ MUELLER.

Witnesses:

CARL GUBLER,  
AUGUST RUEGG.